

# United States Patent Office

2,860,980

Patented Nov. 18, 1958

1

2,860,980

## PLASTICIZATION OF GELATIN WITH DIALKOXY-POLYOXYALKYLENE GLYCOLS

Kirby M. Milton, Rochester, N. Y., assignor to Eastman Kodak Company, Rochester, N. Y., a corporation of New Jersey

No Drawing. Application July 1, 1955  
Serial No. 519,639

7 Claims. (Cl. 96—94)

This invention relates to the plasticization of gelatin and of photographic gelatin emulsions by means of linear polyalkyl ethers.

Some materials such as glycerin or other polyols are known to plasticize gelatin probably because of either their possible interaction with gelatin or their hydroscopicity. The use of sufficient amounts of these polyols to effectively plasticize photographic emulsions at low humidities may be undesirable because of the physical and sensitometric properties they exhibit at high humidities and temperatures. It has been previously recognized that certain polyethylene glycols may be useful in silver halide emulsions to improve static properties, sensitometric properties or coatability. However, there has never been any statement in the art pointing out any unusual value of these glycols for gelatin plasticizing purposes.

One object of my invention is to provide gelatin coating compositions which give coatings having good flexibilities. Another object of my invention is to plasticize photographic gelatin layers and photographic films containing those layers. A further object of my invention is to plasticize gelatin employed for photographic purposes without any adverse physical or sensitometric effects as might result from many currently known gelatin plasticizers.

I have discovered that the above objects may be obtained by incorporating certain linear polyalkyl ethers in aqueous gelatin coating compositions. These ethers (dialkoxy polyoxyalkylene glycols) have the general formula:  $R_1-O-(R_2O)_n-R_3$ , where  $R_1$ ,  $R_2$  and  $R_3$  are saturated, aliphatic hydrocarbon groups and  $n$  is an integer such as from 1 to 9 and preferably 3-4.  $R_1$  and  $R_3$  each may be either methyl or ethyl whereas  $R_2$  may be any saturated aliphatic hydrocarbon group either straight chain or branched and may be from 1 to 3 carbon atoms. One example of a material of this type which has been found to be useful in accordance with my invention is dimethoxytetraethylene glycol. It is desirable that the chain length of the polyether be enough that there is little or no loss by volatilization upon curing or keeping but not so large that the polyether is incompatible with gelatin when dry. In general 5-50% of plasticizer based on the weight of gelatin will be used but the optimum concentration may vary depending upon the particular polyether used. I have found that the use of the dialkoxy polyoxyalkylene glycols for the plasticization of gelatin possesses advantages over the polyoxyalkylene glycols themselves and the monoalkoxy polyoxyalkylene glycols as will be illustrated by the following examples.

### Example 1

Several gelatin sheets were prepared by coating out aqueous solutions of 8% of photographic gelatin and

2

1.6% of plasticizer onto stripping type plates so that gelatin skins with dried thicknesses of 4 mils were obtained. The sheets were cured at 70° F. and 70% R. H. until dry, stripped from the plates, slit to widths of 15 mm. and conditioned to 70° F. and 20% R. H. Folding endurance was tested with an MIT Fold Tester using a tension of 1 kg. and jaws of 0.0155" radius of curvature with a separation of 0.01". Corresponding plasticized silver halide emulsion sheets were also prepared and tested. These tests resulted as follows:

| Percent <sup>1</sup> | Plasticizer                      | MIT Folds at 20% R. H. |                |
|----------------------|----------------------------------|------------------------|----------------|
|                      |                                  | Gelatin Skins          | Emulsion Skins |
| 0                    | None                             | 36                     | 20             |
| 20                   | Glycerin                         | 99                     | 42             |
| 20                   | "Polyethylene Glycol 300"        | 85                     | —              |
| 20                   | "Methoxypolyethylene Glycol 350" | 120                    | 45             |
| 20                   | "Polyethylene Glycol 600"        | 74                     | 55             |
| 20                   | Dimethoxytetraethylene Glycol    | 137                    | 86             |

<sup>1</sup> Parts per 100 parts of gelatin.

### Example 2

Compositions were prepared from a negative type photographic gelatin emulsion using various plasticizers. The resulting emulsions were coated on cellulose acetate support and dried at high temperatures. The films obtained were tested and the following results were obtained.

| Percent | Plasticizer                      | MIT Folds at 10% R. H. |       |      |
|---------|----------------------------------|------------------------|-------|------|
|         |                                  | MIT Folds              | Wedge | Vise |
| 35      | "Polyethylene Glycol 300"        | 0                      | —     | —    |
| 30      | "Methoxypolyethylene Glycol 350" | 1                      | —     | —    |
| 30      | "Polyethylene Glycol 600"        | 5                      | —     | —    |
| 30      | Dimethoxytetraethylene Glycol    | 21                     | —     | —    |

### Example 3

In a similar experiment the proportion of plasticizer was varied. Tests of those films resulted as follows:

| Percent | Plasticizer                   | Brittleness at 10% R. H. |       |      |
|---------|-------------------------------|--------------------------|-------|------|
|         |                               | MIT Folds                | Wedge | Vise |
| 0       | None                          | 0                        | .35   | .11  |
| 20      | Glycerin                      | 0                        | .26   | .03  |
| 20      | Dimethoxytetraethylene Glycol | 19                       | .11   | .02  |

### Example 4

Films were prepared as described above using a positive type photographic emulsion with and without dimethoxytetraethylene glycol as a plasticizer. These films tested as follows:

| Percent | Plasticizer                       | Brittleness at 10% R. H. |       |      |
|---------|-----------------------------------|--------------------------|-------|------|
|         |                                   | MIT Folds                | Wedge | Vise |
| 60      | No plasticizer                    | 6                        | .32   | .22  |
| 60      | 20% Dimethoxytetraethylene Glycol | 44                       | .07   | .04  |

## Example 5

Various photographic emulsions (used to form Kodachrome film) were plasticized, and the resulting compositions were coated one over the other on cellulose acetate support. The resulting plasticized film was compared to a (Kodachrome) commercial photographic film similar in all respects save the lack of emulsion plasticizer in any of the layers. The results obtained were as follows:

| Plasticizer                                     | Brittleness at 10% R. H. |       |      |
|-------------------------------------------------|--------------------------|-------|------|
|                                                 | MIT<br>Folds             | Wedge | Vise |
| No plasticizer                                  | 1                        | .22   | .25  |
| 20% Dimethoxytetraethylene glycol in all layers | 21                       | .07   | .20  |

## Example 6

Films were coated from a photosensitive emulsion without plasticizer and with 20% and 30% of plasticizer respectively. The results obtained were as follows:

|                                   | Brittleness                     |                         |
|-----------------------------------|---------------------------------|-------------------------|
|                                   | MIT<br>Folds at<br>10%<br>R. H. | Vise at<br>14%<br>R. H. |
| No plasticizer                    | 0                               | .28                     |
| 20% Dimethoxytetraethylene Glycol | 22                              | .19                     |
| 30% Dimethoxytetraethylene Glycol | 25                              | .10                     |

## Example 7

Strips of gelatin coatings were prepared in a series of preparations in the manner described above and plasticizers in accordance with our invention and other similar compounds were used in both gelatin per se and in photographic emulsion compositions in the proportion of 20 parts per 100 parts of gelatin.

| Plasticizer<br>$R_1-O-(R_2O)_n-R_3$ |     |          | MIT Folds at 20%<br>R. H. |          |
|-------------------------------------|-----|----------|---------------------------|----------|
| $R_1$                               | $n$ | $R_3$    | Gelatin                   | Emulsion |
| H                                   | 4   | H        | 36                        | 38       |
| H                                   | 4   | $C_2H_5$ | 48                        | 50       |
| $CH_3$                              | 3   | $CH_3$   | 57                        | 64       |
| $CH_3$                              | 4   | $CH_3$   | 62                        | 85       |

The use of the dialkoxy ethers of polyoxyalkylene glycols in amounts up to 20-30% or even more in gelatin coating compositions based on the weight of the gelatin was found to have no derogatory effect upon the properties of photographic emulsions such as coefficients of friction, wash water melting points, humidity curl amplitudes, mushiness, ferrotyping and abrasion resistance of the films. In the examples given other dialkoxy ethers of glycols may be used to plasticize gelatin. For instance, any one of the following compounds may be employed by the methods described in the example with similar results: dimethoxytetraoxyethylene glycol, dimethoxy-pentaoxyethylene glycol, dimethoxyhexaoxyethylene glycol, dimethoxytetraoxypropylene glycol, diethoxytetraoxyethylene glycol, diethoxypropylene glycol, diethoxytetraoxyisopropylene glycol, diethoxytriaxyethylene glycol, dimethoxytriaxypropylene glycol, dimethoxypenta-oxyethylene glycol, dimethoxyhexaoxyethylene glycol.

If thought desirable, gelatin compositions, instead of being plasticized entirely with the dialkoxy ethers of

polyoxyalkylene glycols as described herein, may be plasticized with mixtures of one or more of those compounds with compatible glycols providing at least 50% of the plasticizing material is the dialkoxy ether of a polyoxyalkylene glycol. As examples of mixtures which may be useful are compositions of dimethoxytetraoxyethylene glycol with glycerin, mixtures of dimethoxy tetraoxyethylene glycol with polytriethylene glycols or mixtures of dimethoxytriaxyethylene glycol with glycerin, triethylene glycol or ethylene glycol, providing the ether of the polyoxyalkylene glycol is at least 50% of the plasticizer employed in the gelatin composition.

Ordinarily the plasticizers will be added to the gelatin solution before the formation of a coating thereof. However, where a multi-layer coating is desired, plasticization can be accomplished by incorporating a plasticizer in accordance with my invention into one of the gelatin layers which plasticizer migrates into layers adjacent thereto. The plasticizers in accordance with my invention are free of the disadvantages common in gelatin plasticizers containing hydroxyl groups such as poor flexibilities at low humidities, abnormally high moisture intake and possibly undesirable sensitometric properties at high humidity.

I claim:

1. A plasticized gelatin composition comprising gelatin mixed with 5-50% of a plasticizing material at least 50% of which is a dialkoxy polyoxyalkylene glycol having the formula:



where  $R_1$  and  $R_3$  are alkyl groups of 1-2 carbon atoms,  $R_2$  is a saturated aliphatic hydrocarbon group from 1-3 carbon atoms and  $n$  is an integer within the range of 1-9.

2. A plasticized gelatin composition comprising gelatin and 20-30% of a plasticizing material at least half of which is a dialkoxy ether of a polyoxyalkylene glycol.

3. A plasticized gelatin composition comprising gelatin and 5-50% based on the gelatin of a plasticizer at least 50% of which is dimethoxytetraethylene glycol.

4. A plasticized gelatin composition comprising gelatin and 5-50% based on the gelatin of a plasticizer at least 50% of which is dimethoxytriaethylene glycol.

5. A plasticized gelatin-silver halide photographic emulsion which contains a plasticizer having the formula:



$R_1$  and  $R_3$  being alkyl groups of 1-2 carbon atoms,  $R_2$  being a saturated aliphatic hydrocarbon group of 1-3 carbon atoms and  $n$  being an integer within the range of 1-9.

6. A plasticized gelatin composition comprising gelatin containing a plasticizer having the formula:



$R_1$  and  $R_3$  being alkyl groups of 1-2 atoms,  $R_2$  being a saturated aliphatic hydrocarbon group of 1-3 carbon atoms and  $n$  is 3-4.

7. A plasticized gelatin-silver halide photographic emulsion which contains a plasticizer having the formula:



$R_1$  and  $R_3$  being alkyl groups of 1-2 atoms,  $R_2$  being a saturated aliphatic hydrocarbon group of 1-3 carbon atoms and  $n$  is 3-4.

## References Cited in the file of this patent

## UNITED STATES PATENTS

- 2,240,469 Swan et al. \_\_\_\_\_ Apr. 29, 1941  
 2,286,314 Seymour et al. \_\_\_\_\_ June 16, 1942  
 2,684,909 Leekley et al. \_\_\_\_\_ July 27, 1954

UNITED STATES PATENT OFFICE  
CERTIFICATE OF CORRECTION

Patent No. 2,860,980

November 18, 1958

Kirby M. Milton

It is hereby certified that error appears in the printed specification of the above numbered patent requiring correction and that the said Letters Patent should read as corrected below.

Column 4, line 63, for "1-2 atoms" read -- 1-2 carbon atoms --.

Signed and sealed this 10th day of March 1959.

(SEAL)  
Attest:

KARL H. AXLINE  
Attesting Officer

ROBERT C. WATSON  
Commissioner of Patents